# EUROPEAN PATENT SPECIFICATION

(11) **EP 0 803 879 B1**
(45) Date of publication and mention of the grant of the patent: **24.03.2004**
(21) Application number: 97201655.4
(22) Date of filing: 15.09.1989
(51) Int. Cl.: H01C 7/02

(54) **Conductive polymer composition**
Leitfähige Polymerzusammensetzung
Composition polymère conductrice

(30) Priority: 20.09.1988 US 247059
(43) Date of publication of application: 29.10.1997
(62) Divisional of application: 89910755.1
(73) Proprietor: TYCO Electronics Corporation, Menlo Park, CA 94025-1164 (US)
(72) Inventor: Shafe, Jeff, Redwood City, CA 94063 (US); Straley, O. James, Redwood City, CA 94063 (US); McCarty, Gordon, San Jose, CA 95131 (US); Oswal, Ravinder K., Union City, CA 94587 (US); Trammell, Bernadette A, Menlo Park, CA 94025 (US)
(74) Representative: Jay, Anthony William

(56) References cited:
- EP-A- 0 123 540
- EP-A- 0 235 454
- US-A- 4 237 441
- US-A- 4 277 673
- US-A- 4 591 700
- US-A- 4 668 857

## Description

### BACKGROUND OF THE INVENTION

### Field of the Invention

This invention relates to conductive polymer compositions and electrical devices comprising them.

### Background of the Invention

Conductive polymer compositions and electrical devices such as heaters and circuit protection devices comprising them are well-known. Reference may be made, for example, to U.S. Patent Nos. 3,793,716, 3,823,217, 3,858,144, 3,861,029, 3,914,363, 4,017,715, 4,177,376, 4,188,276, 4,237,441, 4,242,573, 4,246,468, 4,286,376, 4,304,987, 4,318,881, 4,330,703, 4,334,148, 4,334,351, 4,388,607, 4,400,614, 4,425,497, 4,426,339, 4,435,639, 4,459,473, 4,514,620, 4,520,417, 4,529,866, 4,534,889, 4,543,474, 4,545,926, 4,547,659, 4,560,498, 4,571,481, 4,574,188, 4,582,983, 4,631,392, 4,638,150, 4,654,511, 4,658,121, 4,659,913, 4,661,687, 4,667,194, 4,673,801, 4,698,583, 4,719,335, 4,722,758, and 4,761,541, European Patent Publication Nos. 38,718 (Fouts et al, published October 28, 1981), 158,410 (Batliwalla et al, published October 16, 1985), and 231,068 (Barma et al, published August 5, 1989).

Conductive polymer compositions which exhibit PTC (positive temperature coefficient of resistance) behavior are particularly useful for self-regulating strip heaters and circuit protection devices. These electrical devices utilize the PTC anomaly, i.e. an anomalous rapid increase in resistance as a function of temperature, to limit the heat output of a heater or the current flowing through a circuit. Compositions which exhibit PTC anomalies and comprise carbon black as the conductive filler have been disclosed in a number of references. U.S. Patent No. 4,237,441 (van Konynenburg et al.) discloses suitable carbon blacks for use in PTC compositions with resistivities less than 7 ohm-cm. U.S. Patent No. 4,388,607 (Toy et al) discloses appropriate carbon blacks for use in compositions for strip heaters. U.S. Patent No. 4,277,673 (Kelly) discloses self-regulating articles which comprise highly resistive carbon blacks. These blacks, either alone or in combination with a low resistivity carbon black, form PTC compositions which provide significantly shorter annealing times.

As indicated in the references, a large number of carbon blacks are suitable for use in conductive compositions. The choice of a particular carbon black is dictated by the physical and electrical properties of the carbon black and the desired properties, e.g. flexibility or conductivity, of the resulting composition. The properties of the carbon blacks are affected by such factors as the particle size, the surface area, and the structure, as well as the surface chemistry. This chemistry can be altered by heat or chemical treatment, either during the production of the carbon black or in a post-production process, e.g. by oxidation. Oxidized carbon blacks frequently have a low surface pH value, i.e. less than 5.0, and may have a relatively high volatile content. When compared to nonoxidized carbon blacks of similar particle size and structure, oxidized carbon blacks have higher resistivities. It is known that carbon blacks which are oxidized provide improved flow characteristics in printing inks, improved wettability in certain polymers, and improved reinforcement of rubbers.

### SUMMARY OF THE INVENTION

We have now found that conductive polymer compositions with improved thermal stability can be made when the conductive filler comprises carbon black with a low pH. We have found that the use of such carbon blacks results in an increased PTC anomaly when compared to similar, nonoxidized carbon blacks, even when the composition is more highly reinforced due to an increased filler content required to compensate for higher resistibity. Therefore, in one aspect, this invention provides an electrical device which comprises
(I)
   (A) a PTC element comprising a conductive polymer composition which exhibits PTC behaviour, and which comprises:
      (a) at least one organic polymer which has a crystallinity of at least 15%; and
      (b) at least 4% by weight of the composition of a carbon black which has a pH of less than 4.0;
         and wherein the entirety of organic polymer(s) in the conductive polymer composition has an overall crystallinity of at least 5% and a melting point Tₘ; and
   (B) two electrodes which can be connected to a source of electrical power to pass current through the PTC element;
(II) has a resistance Rᵢ at 20°C; and
(III) is such that if it is maintained at Tₘ for 50 hours, and is then cooled to 20°C, it has a resistance at 20°C, from 0.25Rᵢ to 1.75Rᵢ;
   characterised in that
(IV) the electrical device is a circuit protection device;
(V) the conductive polymer composition has a resistivity of 0.1 to 100 ohm-cm;
(VI) the PTC element is a laminar element; and
(VII)the electrodes are metal sheet or conductive paint electrodes attached to the PTC element.

### DETAILED DESCRIPTION OF THE INVENTION

The carbon blacks useful in the conductive polymer compositions of this invention have pH values of less than 4.0, particularly less than 3.0. The pH is a measure of the acidity or alkalinity of the carbon black surface. A pH of 7.0 indicates a chemically neutral surface; values less than 7.0 are acidic, those higher than 7.0 are basic. Low pH carbon blacks generally have a relatively high volatile content, volatile content being a measure of the amount of chemisorbed oxygen which is present on the surface of the carbon black. The amount of oxygen can be increased by oxidation in a post-production process. The resulting carbon black will have a higher surface activity. For purposes of this specification, the terms "low pH carbon black" and "oxidized carbon black" are used as equivalent terms. The pH of the carbon black is that which is measured prior to mixing the carbon black with the polymer.

The low pH carbon blacks of this invention are used in conductive polymer compositions which exhibit PTC (positive temperature coefficient) behavior in the temperature range of interest when connected to a source of electrical power. The terms "PTC behavior" and "composition exhibiting PTC behavior" are used in this specification to denote a composition which has an R₁₄ value of at least 2.5 or an R₁₀₀ value of at least 10, and preferably both, and particularly one which has an R₃₀ value of at least 6, where R₁₄ is the ratio of the resistivities at the end and the beginning of a 14°C range, R₁₀₀ is the ratio of the resistivities at the end and the beginning of a 100°C range, and R₃₀ is the ratio of the resistivities at the end and the beginning of a 30°C range. In contrast, "ZTC behavior" is used to denote a composition which increases in resistivity by less than 6 times, preferably less than 2 times in any 30°C temperature range within the operating range of the heater.

Carbon blacks with suitable size, surface area and structure for use in PTC compositions are well-known. Guidelines for selecting such carbon blacks are found in U.S Patent Nos. 4,237,441 (van Konynenburg et al.) and 4,388,607 (Toy et al.). In general, carbon blacks with a relatively large particle size, D (measured in nanometers), e.g. greater than 18 nm, and relatively high structure, e.g. greater than about 70 cc/100 g, are preferred for PTC compositions.

Carbon blacks which are particularly preferred for compositions of the invention are those which meet the criteria that the ratio of the resistivity of the carbon black (in powder form) to the particle size (in nanometers) is less than or equal to 0.1, preferably less than or equal to 0.09, particularly less than or equal to 0.08. The resistivity of the carbon black in ohm-cm is determined by following the procedure described in Columbian Chemicals Company bulletin "The Dry Resistivity of Carbon Blacks" (AD1078). In this test, 3 grams of carbon black are placed inside a glass tube between two brass plungers. A 5 kg weight is used to compact the carbon black. Both the height of the compacted carbon black and the resistance in ohms between the brass plunger electrodes are noted and the resistivity is calculated. The ratio is useful for carbons which are tested in their powder, not pelletized, form. While most nonoxidized carbon blacks fulfill the requirements of this ratio, the carbon blacks particularly useful in this invention are those which both meet the ratio and have a pH of less than 4.0.

Other conductive fillers may be used in combination with the designated carbon black. These fillers may comprise nonoxidized carbon black, graphite, metal, metal oxide, or any combination of these. When a nonoxidized carbon black, i.e. a carbon black with a pH of at least 5.0, is present, it is preferred that the pH of the nonoxidized carbon black be at least 1.0 pH unit greater than the pH of the oxidized carbon black. It is preferred that the low pH carbon black be present at a level of at least 5% by weight, preferably at least 10% by weight, particularly at least 20% by weight of the total conductive filler, e.g. 25 to 100% by weight of the total conductive filler. For most compositions of the invention, the low pH carbon black comprises at least 4% by weight, preferably at least 6% by weight, particularly at least 8% by weight of the total composition. For compositions which comprise inks, the presence of the solvent is neglected and the content of the solid components, e.g. carbon black and polymer, is considered the total composition.

Commercially available carbon blacks which have low pH values may be used. Alternatively, nonoxidized carbon blacks may be treated, e.g. by heat or appropriate oxidizing agents, to produce carbon blacks with appropriate surface chemistry.

The conductive polymer composition comprises an organic polymer which has a crystallinity of at least 15%, e.g. 20 to 30%. Suitable crystalline polymers include polymers of one or more olefins, particularly polyethylene; polyalkenamers such as polyoctenamer; copolymers of at least one olefin and at least one monomer copolymerisable therewith such as ethylene/acrylic acid, ethylene/ethyl acrylate, and ethylene/vinyl acetate copolymers; melt-shapeable fluoropolymers such as polyvinylidene fluoride, ethylene/tetrafluoroethylene copolymers, and terpolymers of vinylidene fluoride, hexafluoropropylene, and tetrafluoroethylene; and blends of two or more such polymers. (The term "fluoropolymer" is used herein to denote a polymer which contains at least 10%, preferably at least 25%, by weight of fluorine, or a mixture of two or more such polymers.) In order to achieve specific physical or thermal properties for some applications, it may be desirable to blend one crystalline polymer with another polymer, either crystalline or amorphous. When there are two or more polymers in the composition, the blend must have a crystallinity of at least 5%. The crystallinity, as well as the melting point Tₘ are determined from a DSC(differential scanning calorimeter) trace on the conductive polymer composition. The Tₘ is defined as the temperature at the peak of the melting curve. If the composition comprises a blend of two or more polymers, Tₘ is defined as the lowest melting point measured for the composition (often corresponding to the melting point of the lowest melting component).

The composition may comprise additional components, e.g. inert fillers, antioxidants, flame retardants, prorads, stabilizers, dispersing agents. Mixing may be conducted by any suitable method, e.g. melt-processing, sintering, or solvent-blending. Solvent-blending is particularly preferred when the conductive polymer composition comprises a polymer thick film ink. The composition may be crosslinked by irradiation or chemical means.

The conductive polymer composition of the invention is used as part of a PTC element in an electrical device which is a circuit protection device. The resistivity of the composition is dependent on the function of the electrical device, the dimensions of the PTC element, and the power source to be used. The resistivity is, for example, from 0.01 to 100 ohm-cm for circuit protection devices which are powered at voltages from 15 to 600 volts. The PTC element may be of any shape to meet the requirements of the application. Circuit protection devices and laminar heaters frequently comprise laminar PTC elements, while strip heaters may be rectangular, elliptical, or dumbell- ("dogbone-") shaped. When the conductive polymer composition comprises an ink, the PTC element may be screen-printed or applied in any suitable configuration. Appropriate electrodes, suitable for connection to a source of electrical power, are selected depending on the shape of the PTC element. Electrodes may comprise metal wires or braid, e.g. for attachment to or embedment into the PTC element, or they may comprise metal sheet, metal mesh, conductive (e.g. metal- or carbon-filled) paint, or any other suitable material.

The electrical devices of the invention show improved stability under thermal aging and electrical stress. When a device is maintained at a temperature equal to Tₘ for a period of 50 hours, the resistance at 20°C measured after aging, i.e. R_{f50}, will differ from the initial resistance at 20°C, i.e. Rᵢ, by no more than 75%, preferably no more than 60%, particularly no more than 50%, producing an R_{f50} of from 0.25 Rᵢ to 1.75 Rᵢ, preferably from 0.40 Rᵢ to 1.60 Rᵢ, particularly from 0.50 Rᵢ to 1.50 Rᵢ. If a similar test is conducted for 300 hours, the change in resistance will be less than 50%, preferably less than 40%, particularly less than 30%, producing a resistance at 20°C after 300 hours, R_{f300}, of from 0.50 Rᵢ to 1.50 Rᵢ, preferably from 0.60 Rᵢ to 1.40 Rᵢ, particularly from 0.70 Rᵢ to 1.30 Rᵢ. It is to be understood that if a device meets the resistance requirement when tested at a temperature greater than Tₘ, it will also meet the requirement when tested at Tₘ. Similar results will be observed when the device is actively powered by the application of voltage. The change in resistance may reflect an increase or decrease in device resistance. In some cases, the resistance will first decrease and then increase during the test, possibly reflecting a relaxation of mechanically-induced stresses followed by oxidation of the polymer. Particularly preferred compositions comprising fluoropolymers may exhibit stability which is better than a 30% change in resistance.

The invention is illustrated by the following examples.

### Examples 1 to 10

For each example, an ink was prepared by blending the designated percent by weight (of solids) of the appropriate carbon black with dimethyl formamide in a high shear mixer. The solution was then filtered and powdered Kynar™ 9301 (a terpolymer of vinylidene fluoride, hexafluoropropylene, and tetrafluoroethylene with a melting point of about 88°C, available from Pennwalt) in an amount equal to (100 - % carbon black) was added to the filtrate and allowed to dissolve over a period of 24 to 72 hours. (Approximately 60% solvent and 40% solids was used in making the ink). Silver-based ink electrodes (Electrodag™ 461SS, available from Acheson Colloids) were printed onto ethylene-tetrafluoroethylene substrates and samples of each ink were applied. Samples of each ink were aged in ovens at temperatures of 65, 85, 107 and 149°C. Periodically, the samples were removed from the oven and the resistance at room temperature (nominally 20°C), Rₜ, was measured. Normalized resistance, Rₙ, was determined by dividing Rₜ by the initial room temperature resistance, Rᵢ. The extent of instability was determined by the difference between Rₙ and 1.00. Those inks which comprised carbon blacks with a pH of less than 5 were generally more stable than the inks comprising higher pH blacks.

**TABLE I**

| Stability of Conductive Inks After Aging at Elevated Temperature for 300 Hours (Resistance Measured at Room Temperature) | | | | | | |
|---|---|---|---|---|---|---|
| Carbon Example/ Black | pH | Wt% CB | Rₙ @ 65°C | Rₙ @ 85°C | Rₙ @ 107°C | Rₙ @ 149°C |
| 1 Conductex™ SC | 7.0 | 3.0 | 1.22 | 1.75 | 5.61 | 6.39 |
| 2 Raven™ 1500 | 6.0 | 3.0 | 1.01 | 1.92 | 11.88 | 20.0 |
| 3 Raven™ 890 | 6.5 | 6.0 | 1.27 | 1.77 | 2.92 | 6.07 |
| 4 Raven™ 850 | 7.0 | 4.0 | 1.32 | 2.05 | 4.08 | 8.48 |
| 5 Raven™ 1000 | 6.0 | 4.0 | 1.18 | 1.43 | 1.94 | 4.40 |
| 6 Raven™ 16 | 7.0 | 5.6 | 1.11 | 1.89 | - | - |
| 7 Raven™ 5750 | 2.1 | 8.1 | 0.87 | 0.92 | 0.97 | 0.56 |
| 8 Raven™ 1040 | 2.8 | 9.1 | 0.96 | 1.15 | 1.47 | 1.34 |
| 9 Raven™ 1255 | 2.5 | 6.0 | 1.04 | 1.26 | 1.12 | 0.65 |
| 10 Raven™ 14 | 3.0 | 7.0 | 0.82 | 1.00 | - | - |
| Notes to Table I: (1) Conductex and Raven are trademarks for carbon blacks available from Columbian Chemicals. (2) Wt% CB indicates the percent by weight of carbon black used in each ink. (3) Carbon blacks in Examples 1, 2 and 3 produced inks with ZTC characteristics. | | | | | | |

Measurements on two samples at 93°C (i.e. Tₘ + 5°C) showed that after 50 hours Example 6 (pH = 7.0) had an Rₙ of 2.53 and Example 10 (pH 3.0) had an Rₙ of 1.48.

The Rₙ values for Examples 1 to 6 and Examples 7 to 10 were averaged for each time interval at the test temperatures. The results, shown in Table II, indicate that the carbon blacks with high pH values were significantly less stable than those with low pH values.

**TABLE II**

| Average Rₙ Values | | | | | | | | | | | | |
|---|---|---|---|---|---|---|---|---|---|---|---|---|
| Example | Hours @65°C | | | Hours @85°C | | | Hours @107°C | | | Hours @149°C | | |
| | 300 | 675 | 1256 | 300 | 675 | 1256 | 300 | 675 | 1256 | 300 | 675 | 1256 |
| 1 to 6 (pH>5) | 1.2 | 1.2 | 1.2 | 1.8 | 1.8 | 1.9 | 5.3 | 7.9 | 9.0 | 9.1 | 14.2 | 15.6 |
| 7 to 10 (pH<5) | 0.9 | 0.9 | 0.9 | 1.1 | 1.0 | 1.0 | 1.2 | 1.3 | 1.3 | 0.9 | 1.0 | 1.0 |

Additional tests were conducted on samples from Examples 6 and 10 in order to determine the stability of the compositions under applied voltage. After measuring the initial room temperature resistance, the samples were placed in environmental chambers maintained at either 20 or 65°C and appropriate voltage was applied to each sample in order to produce comparable watt densities. Periodically, the voltage was disconnected and the resistance of each sample measured. Rₙ was calculated as previously described. It is apparent from the results in Table III that the samples containing the oxidized carbon black were more stable than those with nonoxidized carbon black.

**TABLE III**

| Rₙ of Samples After Active Testing (Time in Hours) | | | | | | | | | | | | |
|---|---|---|---|---|---|---|---|---|---|---|---|---|
| | pH | Applied Volts | Power (w/in²) | | Rₙ 20°C | | | | Rₙ 65°C | | | |
| | | | Samples at | | | | | | | | | |
| | | | 20°C | 65°C | 300 | 600 | 1000 | 4000 | 300 | 600 | 1000 | 4000 |
| Example 6 Raven™ 16 | 7.0 | 120 | 2.3 | 2.8 | 1.1 | 1.3 | 1.5 | 6.0 | 1.4 | 1.5 | 1.5 | 2.0 |
| Example 10 Raven™ 14 | 3.0 | 240 | 1.9 | 3.1 | 0.8 | 0.8 | 0.8 | 0.7 | 0.9 | 0.8 | 0.7 | 0.8 |

### Examples 11 to 14

Following the procedure of Examples 1 to 10, inks were prepared using Kynar™ 9301 as a binder and incorporating the carbon blacks listed in Table IV. The resistance vs. temperature characteristics were measured by exposing samples of each ink to a temperature cycle from 20°C to 82°C. The height of the PTC anomaly was determined by dividing the resistance at 82°C (R₈₂) by the resistance at 20°C (R₂₀). It was apparent that at comparable resistivity values the PTC anomaly was higher for the oxidized carbon blacks than for the nonoxidized carbon blacks.

**TABLE IV**

| Carbon Example/Black | pH | D (nm) | S.A. (m²/g) | DBP (cc/100g) | R_{CB} (ohm-cm) | R_{CB}/D | Wt% | Rho (ohm-cm) | PTC Height |
|---|---|---|---|---|---|---|---|---|---|
| 11 Raven™ 1000 | 6.0 | 28 | 95 | 63 | 2.46 | 0.088 | 4.0 | 750 | 3.1x |
| 12 Raven™ 1040 | 2.8 | 28 | 90 | 99 | 19.20 | 0.695 | 9.1 | 720 | 13.0x |
| 13 Raven™ 450 | 8.0 | 62 | 33 | 67 | 1.36 | 0.021 | 5.0 | 150 | 23x |
| 14 Raven™ 14 | 3.0 | 59 | 45 | 111 | 4.36 | 0.074 | 12.0 | 100 | 42x |
| Notes to Table IV: (1) D represents the particle size of the carbon black in nm. (2) S.A. represents the surface area of the carbon black in m²/g as measured by a BET nitrogen test. (3) DBP is a measure of the structure of the carbon black and is determined by measuring the amount in cubic centimeters of dibutyl phthalate absorbed by 100 g of carbon black. (4) Wt% represents the percent by weight of the total solids content of the ink that is carbon black. (5) Rho is the resistivity of the ink in ohm-cm. (6) PTC Height is the height of the PTC anomaly as determined by R₈₂/R₂₀. (7) R_{CB} is the dry resistivity of the carbon black in powder form under a 5 kg load. (8) R_{CB}/D is the ratio of the dry resistivity of the carbon black to the particle size. | | | | | | | | | |

### Example 15

Using a Brabender™ mixer, 85% by weight of Kynar™ 9301 was melt-processed with 15% by weight of Raven™ 16. (Raven™ 16 has a pH of 7.0, a particle size of 61 nm, a surface area of 25 m²/g, a DBP of 105 cc/100 g and a dry resistivity of 1.92.) The compound was pelletized and then extruded through a strand die to produce a fiber with a diameter of approximately 0.070 inch (0.18 cm). Silver paint (Electrodag™ 504 available from Acheson Colloids) was used to apply electrodes to pieces of the fiber. The fiber pieces were then tested at 85°C, 107°C, and 149°C following the procedure of Examples 1 to 10. The results are shown in Table V. The test for these samples was discontinued after 743 hours.

### Example 16

Following the procedure of Example 15, 20% by weight of Raven™ 14 was mixed with Kynar™ 9301, extruded into a fiber, and thermally aged. The results as shown in Table V indicate that this oxidized carbon black was more stable on aging than a similar carbon black with a higher pH. When tested at 93°C, i.e. (Tₘ + 5)°C, fibers of Example 15 had an Rₙ after 50 hours of 2.76; those of Example 16 had an Rₙ of 1.73.

**TABLE V**

| Rₙ Values for Extruded Fibers | | | | | | |
|---|---|---|---|---|---|---|
| | Time in Hours | | | | | |
| | 146 | 265 | 743 | 1058 | 1687 | 2566 |
| 85°C: | | | | | | |
| Ex.15 (Raven™ 16) | 2.61 | 3.13 | 3.12 | - | - | - |
| Ex.16 (Raven™ 14) | 1.40 | 1.23 | 1.05 | 1.15 | 1.15 | 1.16 |

| 107°C: | | | | | | |
|---|---|---|---|---|---|---|
| Ex. 15 (Raven™ 16) | 3.95 | 4.40 | 101 | - | - | - |
| Ex. 16 (Raven™ 14) | 0.78 | 0.98 | 1.12 | 0.80 | 1.16 | 1.05 |

| 149°C: | | | | | | |
|---|---|---|---|---|---|---|
| Ex. 15 (Raven™ 16) | 27.6 | 137 | 604 | - | - | - |
| Ex. 16 (Raven™ 14) | 0.65 | 1.07 | 1.52 | 1.43 | 1.91 | 2.83 |

### Example 17

Following the procedure of Example 15, fibers were prepared by blending 55% by weight Elvax™ 250 (ethylene vinyl acetate copolymer with a melting point of 60°C, available from Dow) and 45% by weight Raven™ 22 (carbon black with a pH of 7.0, a particle size of 62 nm, a surface area of 25 m²/g, and a DBP of 113 cc/100 g, available from Columbian Chemicals). An ink was prepared by dissolving the fibers in xylene. After 813 hours at 52°C, the Rₙ value was 0.94.

### Example 18

Following the procedure of Example 17, fibers were first prepared with 50% by weight Raven™ 14 in Elvax™ 250 and were then dissolved in xylene. After 813 hours at 52°C, the Rₙ value of the ink was 0.88.

### Example 19

Fibers were prepared from 76% by weight PFA™ 340 (a copolymer of tetrafluoroethylene and a perfluorovinyl ether with a Tₘ of 307°C, available from du Pont) and 24% by weight Raven™ 600 (carbon black with a pH of 8.3, particle size of 65 nm, DBP of 82 cc/100g, and surface area of 34 m²/g, available from Columbian Chemicals) as in Example 15. Samples tested at 311°C for 50 hours had an Rₙ of 0.55.

### Example 20

Following the procedure of Example 19, fibers were prepared with 17% by weight Raven™ 14. After 50 hours at 311°C, the Rₙ value was 0.93.

## Claims

1. An electrical device which comprises
(I)
(A) a PTC element comprising a conductive polymer composition which exhibits PTC behaviour, and which comprises:
(a) at least one organic polymer which has a crystallinity of at least 15%; and
(b) at least 4% by weight of the composition of a carbon black which has a pH of less than 4.0;
and wherein the entirety of organic polymer(s) in the conductive polymer composition has an overall crystallinity of at least 5% and a melting point Tₘ; and
(B) two electrodes which can be connected to a source of electrical power to pass current through the PTC element;
(II) has a resistance Rᵢ at 20°C; and
(III) is such that if it is maintained at Tₘ for 50 hours, and is then cooled to 20°C, it has a resistance at 20°C from 0.25Rᵢ to 1.75Rᵢ;
**characterised in that**
(IV) the electrical device is a circuit protection device;
(V) the conductive polymer composition has a resistivity of 0.1 to 100 ohm-cm;
(VI) the PTC element is a laminar element; and
(VII)the electrodes are metal sheet or conductive paint electrodes attached to the PTC element.

2. An electrical device according to claim 1, **characterised in that** the carbon black having a pH of less than 4.0 is the sole conductive filler in the conductive polymer composition.

3. An electrical device according to claim 1 or 2, **characterised in that** the carbon black has a pH of less than 3.0.

4. An electrical device according to any one of the preceding claims, **characterised in that** the conductive polymer comprises a polymer thick film ink.

5. An electrical device according to any one of the preceding claims **characterised in that** the conductive polymer has been crosslinked.

6. An electrical device according to any one of the preceding claims, **characterised in that** the composition further comprises (i) carbon black which has a pH which is at least 5.0 or (ii) graphite.

7. An electrical device according to any one of the preceding claims **characterised in that** the polymer is a fluoropolymer.

8. An electrical device according to any one of the preceding claims **characterised in that** the carbon black has a particle size of D nanometers and a dry resistivity R_{CB} such that (R_{CB}/D) is less than or equal to 0.1.

## Patentansprüche

1. Elektrische Vorrichtung, die folgendes aufweist:
(I)
(A) ein PTC-Element, das eine leitfähige Polymerzusammensetzung aufweist, die ein PTC-Verhalten aufweist, und die folgendes umfaßt:
(a) wenigstens ein organisches Polymer, das eine Kristallinität von wenigstens 15% hat; und
(b) wenigstens 4 Gew.-% der Zusammensetzung Ruß, der einen pH-Wert von weniger als 4,0 hat; und
wobei die Gesamtheit des (der) organischen Polymers (Polymeren) in der leitfähigen Polymerzusammensetzung eine Gesamtkristallinität von wenigstens 5% und einen Schmelzpunkt Tₘ hat; und
(B) zwei Elektroden, die an eine elektrische Stromquelle angeschlossen werden können, um Strom durch das PTC-Element fließen zu lassen;
(II) mit einem Widerstand Rᵢ bei 20°C; und
(III) die Vorrichtung so ausgebildet ist, daß sie, wenn sie für 50 Stunden auf Tₘ gehalten, und anschließend auf 20°C abgekühlt worden ist, einen Widerstand bei 20°C von 0,25 Rᵢ bis 1,75 Rᵢ aufweist;
**dadurch gekennzeichnet, daß**
(IV) die elektrische Vorrichtung eine Stromkreisschutzvorrichtung ist;
(V) die leitfähige Polymerzusammensetzung einen spezifischen Widerstand von 0,1 Ohm x cm bis 100 Ohm x cm hat;
(VI) das PTC-Element ein laminares Element ist; und
(VII) die Elektroden Metallblatt- bzw. Metallfolien oder leitfähige Lackelektroden sind, die mit dem PTC-Element verbunden sind.

2. Elektrische Vorrichtung nach Anspruch 1,
**dadurch gekennzeichnet, daß**
der Ruß mit einem pH-Wert von weniger als 4,0 das einzige leitfähige Füllmittel in der leitfähigen Polymerzusammensetzung ist.

3. Elektrische Vorrichtung nach Anspruch 1 oder 2,
**dadurch gekennzeichnet, daß**
der Ruß einen pH-Wert von weniger als 3,0 hat.

4. Elektrische Vorrichtung nach einem der vorhergehenden Ansprüche,
**dadurch gekennzeichnet, daß**
das leitfähige Polymer eine polymere dickflüssige Folientinte aufweist.

5. Elektrische Vorrichtung nach einem der vorhergehenden Ansprüche,
**dadurch gekennzeichnet, daß**
das leitfähige Polymer quervernetzt worden ist.

6. Elektrische Vorrichtung nach einem der vorhergehenden Ansprüche,
**dadurch gekennzeichnet, daß**
die Zusammensetzung ferner
(i) Ruß mit einem pH-Wert von wenigstens 5,0 oder
(ii) Graphit
aufweist.

7. Elektrische Vorrichtung nach einem der vorhergehenden Ansprüche,
**dadurch gekennzeichnet, daß**
das Polymer ein Fluorpolymer ist.

8. Elektrische Vorrichtung nach einem der vorhergehenden Ansprüche,
**dadurch gekennzeichnet, daß**
der Ruß einen Teilchendurchmesser von D nm und trocken einen spezifischen Widerstand R_{CB} hat, so daß (R_{CB}/D) kleiner oder gleich 0,1 ist.

## Revendications

1. Dispositif électrique qui comprend :
(I)
(A) un élément à coefficient de température positif comprenant une composition polymère conductrice présentant un comportement à coefficient de température positif, et comprenant :
(a) au moins un polymère organique ayant une cristallinité d'au moins 15 % ; et
(b) au moins 4 % en masse de la composition d'un noir de carbone ayant un PH de moins de 4,0 ;
et dans lequel la totalité du ou des polymères organiques dans la composition polymère conductrice présente une cristallinité totale d'au moins 5 % et un point de fusion Tₘ ; et
(B) deux électrodes qui peuvent être connectées à une source de courant électrique pour faire passer le courant dans l'élément à coefficient de température positif ;
(II) a une résistance Rᵢ à 20°C ; et
(III)est tel que, s'il est maintenu à Tₘ pendant 50 heures, puis refroidi à 20°C, il présente une résistance à 20°C de 0,25 Rᵢ à 1,75 Rᵢ ;
**caractérisé en ce que**
(IV) le dispositif électrique est un dispositif de protection de circuit ;
(V) la composition polymère conductrice a une résistivité de 0,1 à 100 ohm-cm ;
(VI) l'élément à coefficient de température positif est un élément laminaire ; et
(VII)les électrodes sont des électrodes en tôle métallique ou en peinture conductrice fixées sur l'élément à coefficient de température positif.

2. Dispositif électrique selon la revendication 1, **caractérisé en ce que** le noir de carbone ayant un pH de moins de 4,0 est la seule charge conductrice dans la composition polymère conductrice.

3. Dispositif électrique selon la revendication 1 ou 2, **caractérisé en ce que** le noir de carbone a un pH de moins de 3,0.

4. Dispositif électrique selon l'une quelconque des revendications précédentes, **caractérisé en ce que** le polymère conducteur comprend une encre polymère pour film épais.

5. Dispositif électrique selon l'une quelconque des revendications précédentes, **caractérisé en ce que** le polymère conducteur a été réticulé.

6. Dispositif électrique selon l'une quelconque des revendications précédentes, **caractérisé en ce que** la composition comprend en outre (i) du noir de carbone ayant un pH qui est d'au moins 5,0 ou (ii) du graphite.

7. Dispositif électrique selon l'une quelconque des revendications précédentes, **caractérisé en ce que** le polymère est un fluoropolymère.

8. Dispositif électrique selon l'une quelconque des revendications précédentes, **caractérisé en ce que** le noir de carbone a une taille de particules de D nanomètres et une résistivité à sec R_{CB} telle que (R_{CB}/D) soit inférieur ou égal à 0,1.
